

A. L. CLAPP,  
FIBER WORKING PROCESS AND PRODUCT.  
APPLICATION FILED JULY 16, 1914.

1,148,359.

Patented July 27, 1915.

Fig. 1.



Fig. 3.



Fig. 2.



Witnesses:

James R. Hodder  
R. G. Hersey

Inventor:

Albert T. Clapp,  
by Geo. H. Maxwell,  
Attorney.

# UNITED STATES PATENT OFFICE.

ALBERT L. CLAPP, OF BRAINTREE, MASSACHUSETTS.

## FIBER-WORKING PROCESS AND PRODUCT.

1,148,359.

Specification of Letters Patent. Patented July 27, 1915.

Application filed July 16, 1914. Serial No. 851,347.

*To all whom it may concern:*

Be it known that I, ALBERT L. CLAPP, a citizen of the United States, and resident of Braintree, county of Norfolk, State of Massachusetts, have invented an Improvement 5 in Fiber-Working Processes and Products, of which the following description, in connection with the accompanying drawings, is a specification, like numerals on the drawings representing like parts.

10 My present invention relates to a novel fiber product, and the process or method of working fiber, and more particularly to the expansion of sheets of fiber for use in the arts, as a plaster backing, wicker basket-work substitute, racks, shelves, novelties, etc.

15 The manufacture of fiber from wood pulp presents a very strong tenacious sheet of any desired thickness. Furthermore, this sheet 20 of fiber may be rendered readily fire proof by the addition of asbestos or sodium silicate precipitation, or magnesia, such fire proofing being readily effected by mixing 25 with the fiber pulp in a beater during the process of manufacture. I have discovered 30 that, by treating such fiber as it is rolled into sheets, and while still wet, pliable, and plastic, by alternately forming a plurality 35 of cuts or slits entirely through such sheet, and then expanding the same, as by running 40 the sheets so cut and slit over expansion devices, rollers, or the like, thus greatly expanding the width of the original sheet, I 45 can produce a fire proof material which, when dried and hardened, will be strong, 50 firm, and tenacious for use in the arts. Such an expanded fiber sheet is of special 55 value, for example, as a fire proof plaster 60 lath. As is well known, the ordinary 65 wooden lath for use in plaster work, particularly in exterior plaster work, on cement 70 buildings, houses, etc., is extremely unsatisfactory, since such plaster work has to be 75 continually and thoroughly wet down, in 80 order to cause a homogeneous surface and 85 the constant expansion and contraction of 90 the wooden lath is deleterious to the plaster 95 wall. The use of metal or wire lath is also 100 50 very unsatisfactory, as metal oxidizes and 105 the repeated moistening operations tend to 110 rust and disintegrate the metal, which 115 weakens it, and quickly shows through the 120 plaster wall in disagreeable stains and 125 55 orings. Under the influence of fire also, 130 wooden lath quickly burns and metal lath

warps, twists, and fails to hold the plaster 135 applied thereto. My fiber lath being uniformly fire proof, water proof, and of great 140 strength and thickness, obviates the difficulties 145 above mentioned, and also provides a 150 cheap material for the uses above mentioned.

155 Referring to the drawings, Figure 1 illustrates in plan view a fragmentary section of 160 an expanded fiber sheet, suitable for use 165 as a fiber lath for buildings; Fig. 2 is a view in cross section of the fiber sheet, before it is expanded, and after the cuts or 170 slits have been formed therein; and Fig. 3 175 is a short sectional plan view of the fiber before 180 it is expanded.

185 I may use any sort of fiber desired, that 190 being made from ordinary wood pulp being 195 inexpensive and well suited for my process 200 and product, particularly when said fiber is 205 treated with a fire proofing material, as 210 above explained. The fiber pulp being 215 turned out in sheets 1 by any well known 220 apparatus is at once subjected to a plurality 225 of cutting actions, such cuts being indicated 230 at 2 in Fig. 2, and are preferably also of 235 equal lengths and overlapping or staggered, 240 being spaced apart as shown in Fig. 3. This 245 operation is performed while the fiber sheet 250 is still wet and plastic, and preferably just 255 after its being rolled into final sheet form. 260 If desired, a plurality of reinforced sections 265 3 may be rolled in the sheet. The sheet of 270 fiber is then led over expanding devices 275 which will draw the entire sheet widthwise 280 to open the cut portions 2 into openings 285 4 as illustrated in Fig. 1, this expanding 290 action also being preferably performed as a 295 continuous operation immediately after the 300 cutting of the slits 2 and while the sheet of 305 fiber material is being rolled out. The 310 extent of the widthwise expansion of the fiber 315 sheet may be varied to suit different types 320 of work, and will be also governed some- 325 what by the length of the slits 2 as will be 330 readily understood. The cuts or slits 2 are 335 also formed to leave suitable webs 5 in the 340 completed product to give desired strength 345 to the sheet, the reinforcing sections 3 add- 350 ing thereto. The fiber sheet 1 will be held 355 expanded or conveyed in this expanded con- 360 dition until it is sufficiently set or dried to 365 retain its shape when the hardening and dry- 370 ing process is completed.

375 I am thus enabled to provide a fire proof 380 fiber lath which will be peculiarly suitable

for plaster work and which will neither expand nor shrink with the application of moisture or the moistened plaster thereto, which will be fireproof and consequently 5 maintain the plaster wall intact during high degree of heat, which will afford a plaster backing incapable of oxidizing, and hence will not discolor the work. Furthermore, such fiber lath may be readily affixed to 10 studding by nails driven therethrough at any point, in much the same manner and with as great ease as is wooden lath, together with all the advantages of length, and rapidity of building construction, which 15 is found in wire or metal lath.

While a principal advantage of my improved process and product consists in affording a fire proof fiber lath, it will also be appreciated that fire proof expanded fiber 20 shelves, partitions, and the like, may be formed therefrom, such fiber sheets being readily cut with an ordinary hand saw, knife, etc., and fitted in any manner desirable. I believe that my process of cutting 25 and preparing fiber sheets while wet and plastic, and then expanding the same while in such wet and plastic condition, is a distinct novelty and I wish to claim the same broadly. It is also believed that an expanded fiber product is broadly new, and that I am entitled to claim the same. It will 30 be understood that such expanded fiber may be finished either as "hard fiber" or as "soft

fiber," it may also be molded into curved sections, corner pieces, or the like, and that it 35 will be serviceable in other uses than those above outlined.

Having described my invention, what I 40 claim as new and desire to secure by Letters Patent is:

1. The process of making expanded fiber, which consists in cutting through sheets of fiber while the same is wet and plastic, and immediately thereafter expanding the fiber sheet widthwise to open the said cuts, and 45 holding the sheet so expanded until dried.

2. The process of making expanded fiber, which consists in making a plurality of staggered longitudinal cuts entirely through the fiber sheet while the same is wet and plastic, 50 and immediately thereafter expanding the fiber sheet widthwise to open the said cuts, and holding the sheet so expanded until dried.

3. As an article of manufacture, an expanded sheet of fiber material, consisting of longitudinal zigzag strips integrally connected. 55

In testimony whereof, I have signed my name to this specification, in the presence of 60 two subscribing witnesses.

ALBERT L. CLAPP.

Witnesses:

JAMES R. HODDER,  
R. J. HERSEY.

Copies of this patent may be obtained for five cents each, by addressing the "Commissioner of Patents, Washington, D. C."